

H. G. SLINGLUFF,  
PROCESS OF DRAWING SHEET GLASS,  
APPLICATION FILED MAY 22, 1919.

1,376,975.

Patented May 3, 1921.

FIG.1.



FIG.2.



INVENTOR  
H. G. Slingluff  
by  
Anna C. Bradley  
Atty.

# UNITED STATES PATENT OFFICE.

HARRY G. SLINGLUFF, OF MOUNT VERNON, OHIO, ASSIGNOR TO PITTSBURGH PLATE GLASS COMPANY, A CORPORATION OF PENNSYLVANIA.

## PROCESS OF DRAWING SHEET-GLASS.

1,376,975.

Specification of Letters Patent. Patented May 3, 1921.

Application filed May 22, 1918. Serial No. 298,966.

To all whom it may concern:

Be it known that I, HARRY G. SLINGLUFF, a citizen of the United States, and a resident of Mount Vernon, in the county of Knox 5 and State of Ohio, have made a new and useful Invention in Processes of Drawing Sheet-Glass, of which the following is a specification.

The invention relates to the drawing of 10 glass in the form of sheets and has to do primarily with a procedure whereby the edges of the sheet in process of generation are maintained in position and prevented from working inward and narrowing the 15 sheet as the drawing progresses. The invention has for its principal object the provision of a simple means of procedure which may be carried out by hand manipulation or by an automatic device whereby 20 the position of the edges of the sheet being drawn are maintained in their proper position throughout the draw and their thickness regulated, thus securing a sheet of continuously uniform width. The procedure is 25 illustrated in the accompanying drawings, wherein:

Figure 1 is a transverse section through a forehearth or drawing tank from which a sheet of glass is being drawn in accordance 30 with my invention; Fig. 2 is a plan view of the apparatus of Fig. 1; Fig. 3 is an enlarged side elevation view showing one edge of the sheet and illustrating the step of the process in which the invention particularly 35 resides; Fig. 4 is a plan view of the sheet and bath illustrated in Fig. 3, and Fig. 5 is a perspective view showing a modified form of tool for carrying out the operation.

Figs. 1 and 2 illustrate the drawing apparatus and operation similar to that illustrated in my pending application Serial No. 225,190, filed March 28th, 1918. In carrying out this operation a sheet of glass is drawn from a forehearth or tank containing 40 a relatively large deep body of glass, and in order to maintain the width of the sheet being drawn, pockets of relatively cooler glass are provided at the sides of the furnace, such pockets of glass serving as viscous 45 bonds between the edge of the sheet and the clay work of the blocks. It has been found in the use of this apparatus that particularly in the initial stages of the formation 50 of the sheet, there is a tendency of the edges 55 to draw in and thicken, and it is the purpose

of this invention to provide means whereby this tendency is counteracted and the edges of the sheet maintained in their proper positions and maintained at proper thickness.

I have found that this object can be accomplished by the use of the cooling tool or rod by which the glass adjacent the edges of the sheet is treated at intervals, depending upon the conditions. Briefly stated, this treatment consists in pressing the end of the 60 tool into the glass on either side of the edge which it is desired to maintain in position. The end of the tool is preferably curved or rounded and is pressed into the glass first 65 on one side of the edge of the sheet and then 70 on the other, the tool at such time being drawn outwardly, so that elongated depressions are produced on each side of the edge. This operation not only thins the edge, but 75 also cools it and by making the glass more viscous, tends to prevent any inward movement of the edge.

The manner in which the invention is practised will be understood by reference to the drawings, which illustrate the procedure 80 in a simple and more or less diagrammatic manner, only so much of the apparatus employed being illustrated as is necessary to make clear the method of operation. Figs. 1 and 2 illustrate a portion of the drawing 85 tank or forehearth with the lower portion of the sheet which is being drawn, the bait and other drawing apparatus for continuously drawing the sheet not being illustrated. In this construction 1 is the tank 90 containing the molten mass of glass 2, and 3 is the sheet being drawn with its edges in proximity to the drawing blocks 4. These drawing blocks are provided with recesses or pockets 5, which are filled with glass 95 normally somewhat cooler than the glass in the main body of the tank.

The extreme edge of the sheet is shown in enlarged detail in Figs. 3 and 4, and it is to this portion of the glass that the tool for 100 maintaining the edge in position is applied. This tool is in the form of a rod of iron 6, preferably about five or six feet long and having its end curved as indicated at 7 in Fig. 3. In the use of the tool the end 7 is 105 pressed into the glass on either side of the edge of the sheet forming the recesses 8. These recesses or pockets may vary in size and dimension but are ordinarily one or two inches deep and perhaps three inches 110

long. They are formed by pressing the end of the tool into the glass and then moving it outward. These depressions or pockets are formed close to the sides of the edge so 5 that the portion 9 (Fig. 4) is somewhat thinned, while the outward movement of the tool tends to pull this edge of the sheet outward slightly. The glass from which the edge is drawn, and particularly the portion 10 (Fig. 4) is cooled by the application of the tool and by exposure to the cooling action of the air, thus making the glass from which the edge of the sheet is formed, more viscous, and in this way tending to maintain 15 the width of the sheet and increase the stiffness of the glass between the edge of the sheet and the clay of the drawing block 4. The recesses may be parallel to the plane of the sheet but are ordinarily somewhat inclined as indicated in Fig. 4.

The tool is preferably used more frequently at the beginning of the drawing, at which time such tool may be used first on one side of the sheet and then on the other 25 about every half minute. As the drawing progresses the frequency at which the tool must be used decreases and after a considerable lapse of time the conditions in the bath may become so established and stabilized 30 that the tool need be used only at long intervals. The portion of the bath from which the drawing of the edges occurs, is relatively stiff, so that the depressions 8 remain in the glass a considerable length of 35 time, although in most cases they have about disappeared when the time arrives for using the tool again.

The tool has been used in most cases in connection with drawing blocks such as 40 those indicated in Figs. 1 and 2, but the operation is not restricted to use in connection with blocks of this type, the procedure having the same function and utility with respect to maintaining the width of the sheet 45 regardless of the type of tank and drawing blocks which are employed. The recesses 8 are preferably not formed at the same time, the tool being used first on one side and then on the other, as heretofore described, 50 but if desired, a tool may be employed such as illustrated in Fig. 5, wherein the handle

portion 11 is provided with a pair of ends 12, so that two recesses may be formed at the same time. The invention is also not limited to the formation of the recesses or 55 pockets by a hand operated tool, as a tool may be used which is power operated, and which makes engagement with the glass at predetermined intervals. Such a tool would preferably have an end approximating in 60 shape that used on the hand tool, but such shape might be varied, depending upon conditions and depending upon the movement given to the tool. Obviously a tool such as that shown in Fig. 5 might also be 65 operated by power means automatically.

What I claim is:

1. In the process of drawing a glass sheet from a molten bath, the step of maintaining the position of the edge of the sheet 70 which consists in depressing elongated recesses or pockets at intervals in the body of molten glass with a cooling tool on each side of the edge and in close proximity thereto.

2. In the process of drawing a glass sheet 75 from a molten bath, the step of maintaining the position of the edge of the sheet which consists in pressing a cooling tool into the body of molten glass at intervals on either side of said edge in close proximity thereto. 80

3. In the process of drawing a glass sheet from a molten bath, the step of maintaining the position of the edge of the sheet which 85 consists in pressing a cooling tool into the body of molten glass at intervals on either side of said edge in close proximity thereto, said tool being given a downward and outward movement tending to thin the edge and move it outwardly.

4. In the process of drawing a glass sheet 90 from a molten bath, the step of maintaining the position of the edge of the sheet which consists in pressing a cooling tool into the body of molten glass at intervals on either side of said edge in close proximity thereto, 95 thus providing a pair of cooling recesses in the glass with a ridge of glass therebetween constituting a lateral extension of such edge.

In testimony whereof, I have hereunto subscribed my name this 14th day of May, 100 1919.

HARRY G. SLINGLUFF.